

United States Patent [19]  
Haack

[11] 3,915,716  
[45] Oct. 28, 1975

[54] CHEMICAL NICKEL PLATING BATH  
[75] Inventor: Wolf-Dieter Haack, Berlin, Germany  
[73] Assignee: Schering AG, Berlin and Bergkamen, Germany  
[22] Filed: Mar. 18, 1970  
[21] Appl. No.: 20,828

2,822,294 2/1958 Gutzeit et al. .... 106/1 X  
2,916,401 12/1959 Puls ..... 106/1 X  
3,024,134 3/1962 Nixon et al. .... 106/1 X  
3,198,659 8/1965 Levy ..... 106/1 X  
3,370,974 2/1968 Hepfer ..... 106/1 X  
3,403,035 9/1968 Schneble et al. .... 106/1 X  
3,438,798 4/1969 Baudrand..... 106/1 X

OTHER PUBLICATIONS

Schwartz, M., Proc. Amer. Electroplating Society, Vol. 47 (1960), pp. 176-183.

Primary Examiner—Lorenzo B. Hayes  
Attorney, Agent, or Firm—Joseph F. Padlon

[30] Foreign Application Priority Data  
Apr. 17, 1969 Germany..... 1920152  
[52] U.S. Cl..... 106/1; 117/47 A; 117/130 E;  
117/160 R  
[51] Int. Cl.<sup>2</sup>..... C23C 3/02  
[58] Field of Search..... 106/1; 117/130 E, 130,  
117/160, 47 A

[56] References Cited  
UNITED STATES PATENTS

2,430,581 11/1947 Pessel ..... 106/1 X

[57] ABSTRACT

A chemical nickel plating bath containing hydrazine or its salts for precipitating nickel coatings in a substrate and having catalytic or corrosion inhibiting properties.

1 Claim, No Drawings

### CHEMICAL NICKEL PLATING BATH

The invention relates to a chemical nickel plating bath containing hydrazine or its salts for precipitating nickel coatings having corrosion inhibiting or catalytic properties.

Nickel coatings can be deposited from known baths by chemical reduction, that is, without an external current source. These baths contain a nickel salt, a reducing agent, complex forming agents and other addition agents in the dissolved state, and they deposit nickel on the base metal upon contact with a catalytically activated surface of the metal.

It is possible to coat not only catalytically active metals in this manner, but also many inactive metals and even non-conductors after previous activation treatment, for example, with palladium nuclei.

The reduction of nickel compounds with sodium hypophosphite has been known for the longest time. Depending on experimental conditions, the coatings so deposited contain 3 - 13% phosphorus. They have the disadvantage of having a lower melting point and a much smaller electric conductivity than pure nickel deposits. Also, they readily become passive and are therefore difficult to reinforce by galvanic deposition because the adherence of the galvanic face coating is low. Moreover, hypophosphite baths are not stable and tend to decompose. It is also difficult to maintain the electrolyte for extended periods because phosphite accumulates as a reaction product, and sparingly soluble nickel phosphite is precipitated. The suspended nickel phosphite causes rough coatings and ultimately decomposition of the bath.

It is further known that nickel salts can be reduced by means of sodium borohydride and of borazanes. The coatings deposited contain 5 - 7% boron in addition to the nickel. However, it is noted that the low melting point and the small electrical conductivity of the nickel-boron alloys are disadvantages. Moreover, the nickel baths containing sodium borohydride can be regenerated only to a limited extent. A borate which formed as a reaction product accumulates in the electrolyte, and interferes with nickel deposition. A special disadvantage of sodium borohydride as a reducing agent is its rapid hydrolysis in the nickel bath. Because this reaction takes place independently from the nickel deposition, the yield of the reaction, based on sodium borohydride, decreases materially with the decreasing use of the bath.

A chemical nickel bath containing a nickel salt, a complexing agent, buffering compounds, hydrazine or its derivatives, and optionally alkali metal hydroxide has been described in U.S. Pat. No. 3,198,659. The bath is operated at a pH value of 6.5 to 11 and at a temperature of 70° to 100°C, preferably 90° to 95°C. Ammonium carbonate may be added to the bath as a complexing agent and buffering compound in amounts of 0.01 or 0.02 mole per liter. There is no suggestion, however, that greater amounts of this compound be used, nor that the pH value be increased beyond the indicated maximum limit. However, under the described conditions, the deposition rate of the nickel is very low and the stability of the bath is unsatisfactory. Because the bath is operated at relatively high temperatures, it is not well suited to the nickel coating of plastics.

According to the invention, nickel coatings having corrosion inhibiting and/or catalytic effects are obtained from a bath which has a high deposition rate and

is extremely stable. As the known bath, the bath of the invention contains an aqueous solution of nickel salt, complexing agent, hydrazine or its salts, and optionally alkali metal hydroxide, as a buffering compound; however, at least one water soluble salt of phosphoric acid or carbonic acid with inorganic or organic bases in concentrations above 0.05 mole per liter, and preferably between 0.05 and 1.0 mole/liter are used, and it has a pH value higher than 11.

A pH value which is higher than that of the known bath and the higher concentration of the above-mentioned buffering compounds in the bath of the invention as compared to the known bath provide substantial advantages and constitute a major advance in the art.

Corrosion resistant nickel coatings of great hardness can be deposited with the bath of the invention on metals and on non-conductors. These nickel layers do not tend to turn passive when they are reinforced by galvanic deposition.

It is also possible to produce nickel coatings having remarkable catalytic effects which are suitable particularly as hydrogenation and dehydrogenation catalysts. They can be deposited on metallic surfaces of any desired shape and, in addition to good adherence, have the advantage of not being pyrophoric.

The bath of the invention additionally permits nickel to be deposited already at a bath temperature above 50°C. The deposition rate is very high, and the stability of the bath is excellent. The upkeep of the electrolyte thus does not present any problems. It is another significant advantage that the electrolyte can be regenerated indefinitely with suitable, concentrated stock solutions of the individual ingredients.

Suitable water soluble salts of phosphoric acid and carbonic acid include, for example, the sodium, potassium, ammonium and hydrazonium salts.

The coatings deposited from the bath with the use of phosphates as buffering compounds generally are of better quality than the coatings obtained with the use of carbonates. The stability of the bath and the nickel deposition rate are more improved by phosphates than by carbonates.

The concentration of the aforementioned phosphates and carbonates is in the range above 0.05 mole/liter, preferably between 0.05 to 1.0 mole/liter.

The aforementioned buffering agents increase not only the deposition rate of the nickel and the stability of the bath, but have the additional advantage to achieve a better adjustment and maintenance of the optimal pH value when used in the aforementioned concentrations, than is possible with the known system. They also cause high solubility of the nickel salts in the bath.

Useful nickel salts include, for example, nickel chloride, nickel sulfate, nickel acetate and others which are employed in concentrations of 0.01 to 0.5 mole/liter.

Hydrazine and its salts, for example, hydrazine sulfate, are employed as reducing agents. The concentration of the reducing agent is about 0.01 to 4.0 moles/liter, based on the hydrazine content.

As is well known, nickel salts can be held in solution in an alkaline medium only by complexing agents. In order to make the desired high deposition rate of nickel possible, the nickel complexes must be neither too stable nor too inert.

Complexing agents particularly suitable for this purpose are, for example, ammonia, amino alcohols and the salts of diphosphoric acid, such as  $\text{Na}_4\text{P}_2\text{O}_7$ , in concentrations of about 0.01 to 4.0 moles/liter.

It is possible to use ammonia as a complexing agent even at elevated temperatures regardless of its volatility when the electrolyte is suitable covered. The usual cover of floating solid bodies, however, is not sufficient. It has been found advantageous to cover the bath with an inert agent insoluble in the liquid of the bath, preferably an aliphatic or aromatic hydrocarbon, such as decalin, or an ether of low volatility, such as di-n-butyl ether.

Objects of metal or ceramics which are first moistened with water can be entered into the bath through the cover layer without the cover layer adhering to them. Organic synthetic resins, however, are generally wetted by the floating covering layer and can thereafter not be coated with nickel.

The bath of the invention is prepared in a manner known in itself, preferably, however, by mixing the components in the following sequence: water, nickel salt, complexing agent, phosphate or carbonate, hydrazine or its salt. Ultimately, the pH is adjusted to the desired value or more than 11 if necessary, for example, by addition of alkali metal hydroxides such as sodium hydroxide.

The bath of the invention may have the following composition: 0.01 to 0.5 mole/liter nickel salt, 0.01 to 4.0 moles/liter complexing agent, 0.01 to 4.0 moles/liter hydrazine or a corresponding amount of a hydrazine salt, between 0.05 and 1.0 mole/liter of a water soluble salt of phosphoric or carbonic acid, and optionally up to 3 mole/liter alkali metal hydroxide, in aqueous solution.

The bath is used in a manner known in the art. Also, this bath is particularly well suited for nickel plating plastic surfaces.

The necessary pretreatment and activation of the plastic surfaces is carried out in the usual manner. Many organic synthetic resin compositions can be roughened by etching, for example, with hot chrome sulfuric acid. The etched plastics are subsequently dipped in a solution of a noble metal salt, for example, palladium chloride, and thereafter in a reducing agent, for example, hydrazine. The activated plastics are then rinsed, and subsequently nickel plated in the chemical nickel plating bath. A nickel plating bath containing a diphosphate, such as  $\text{Na}_4\text{P}_2\text{O}_7$ , is particularly suitable for nickel plating organic synthetic resin compositions or plastics. Nickel is already deposited at the low bath temperature of over 50°C.

At lower bath temperatures, however, the nickel deposition on plastic surfaces activated by means of palladium nuclei starts only after a fairly long induction period.

As has further been found, this induction period can be substantially shortened by the addition of a very small amount of alkali metal hypophosphite, such as sodium hypophosphite, to the nickel plating bath. Simultaneously, complete nickel coating of the plastics and good adhesion of the nickel deposits are achieved. The preferred concentration of the hypophosphite is in the range between approximately 0.002 and 0.1 mole/liter.

According to the invention, hydrazine-bearing nickel baths are already stabilized and excellently by the addi-

tion of phosphates or carbonates. Further stabilization is possible by adding certain inhibitors in low concentrations. Particularly suitable inhibitors are the water soluble salts of lead, cadmium, bismuth, thallium or tin with inorganic or organic acids, or metal cyanides, preferably alkali metal cyanides, in preferred concentrations of  $10^{-6}$  to  $10^{-3}$  mole/liter.

According to a further embodiment of the invention, the bath may additionally contain water soluble salts of cobalt, germanium, tin or thallium in concentrations of about  $10^{-4}$  to  $10^{-2}$  mole/liter. Suitable salts are, for example, the chlorides and sulfates. The deposition conditions are analogous to those of nickel. The alloys obtained from the baths of this composition are distinguished by their superior catalytic activity.

The following Examples further describe and illustrate baths according to the invention.

#### EXAMPLE 1

0.1 Mole/liter nickel (II) chloride  
2.0 Mole/liter ammonia  
0.4 Mole/liter hydrazine  
 $10^{-5}$  Mole/liter lead (II) acetate as stabilizer  
0.4 Mole/liter dipotassium hydrogen phosphate  
pH 12.6; adjusted with sodium hydroxide  
Cover layer: di-n-butyl ether  
Deposition rate: 3.7  $\mu\text{m}/\text{hr}$  at 50°C  
Appearance of nickel layer: light brown, dull

#### EXAMPLE 2

0.1 Mole/liter nickel (II) chloride  
3.0 Mole/liter ammonia  
0.4 Mole/liter hydrazine  
0.4 Mole/liter dipotassiumhydrogen phosphate  
 $3 \times 10^{-6}$  Mole/liter potassium cyanide as stabilizer  
pH 12.2; adjusted with sodium hydroxide  
Cover layer: decalin  
Deposition rate: 15.6  $\mu\text{m}/\text{hr}$  at 80°C  
Appearance of nickel layer: dark brown, dull

#### EXAMPLE 3

0.05 Mole/liter nickel (II) sulfate  
0.2 Mole/liter sodium diphosphate ( $\text{Na}_4\text{P}_2\text{O}_7$ )  
0.2 Mole/liter hydrazine  
0.4 Mole/liter sodium carbonate  
 $10^{-5}$  Mole/liter bismuth (III) nitrate as stabilizer  
pH 11.1  
Deposition rate: 5.4  $\mu\text{m}/\text{hr}$  at 70°C  
Appearance of nickel layer: gray, dull

#### EXAMPLE 4

0.05 Mole/liter nickel (II) sulfate  
0.2 Mole/liter sodium diphosphate ( $\text{Na}_4\text{P}_2\text{O}_7$ )  
0.4 Mole/liter hydrazine  
0.4 Mole/liter dipotassium hydrogen phosphate  
 $10^{-5}$  Mole/liter potassium cyanide as stabilizer  
pH 11.1; adjusted with sodium hydroxide  
Deposition rate: 16.7  $\mu\text{m}/\text{hr}$  at 90°C  
Appearance of nickel layer: brown, bright

#### EXAMPLE 5

0.05 Mole/liter nickel (II) sulfate  
0.2 Mole/liter sodium diphosphate ( $\text{Na}_4\text{P}_2\text{O}_7$ )  
0.6 Mole/liter hydrazine  
0.4 Mole/liter dipotassium hydrogen phosphate  
 $10^{-4}$  Mole/liter tin (II) chloride as stabilizer  
pH 12.0; adjusted with sodium hydroxide

Deposition rate: 7.6  $\mu\text{m}/\text{hr}$  at 70°C  
Appearance of nickel layer: light, bright

## EXAMPLE 6

0.03 Mole/liter nickel (II) sulfate  
0.3 Mole/liter sodium diphosphate ( $\text{Na}_4\text{P}_2\text{O}_7$ )  
0.4 Mole/liter hydrazine  
0.4 Mole/liter dipotassium hydrogen phosphate  
0.008 Mole/liter sodium hypophosphite  
10<sup>-5</sup> Mole/liter cadmium (II) sulfate as stabilizer  
pH 12.0; adjusted with sodium hydroxide  
Deposition rate: 3  $\mu\text{m}/\text{hr}$  at 60°C  
Appearance of nickel layer: light, bright  
This electrolyte may also be used for nickel plating plastics.

## EXAMPLE 7

0.05 Mole/liter nickel (II) chloride  
1.5 Mole/liter monoethanolamine  
0.4 Mole/liter hydrazine  
0.4 Mole/liter dipotassium hydrogen phosphate  
3 $\times$ 10<sup>-5</sup> Mole/liter thallium (I) sulfate  
pH 11.7; adjusted with sodium hydroxide  
Deposition rate: 8.0  $\mu\text{m}/\text{hr}$  at 70°C  
Appearance of nickel layer: brown, semi-bright

## EXAMPLE 8

0.05 Mole/liter nickel (II) sulfate  
0.005 Mole/liter cobalt (II) sulfate  
0.2 Mole/liter hydrazine  
0.4 Mole/liter dipotassium hydrogen phosphate  
0.2 Mole/liter sodium diphosphate ( $\text{Na}_4\text{P}_2\text{O}_7$ )  
From this electrolyte, when adjusted to pH 11.4 (with sodium hydroxide), and at a temperature of 70°C, a coating was deposited on a steel sheet. This deposit is distinguished by remarkable catalytic activity.

The catalytic activity was determined by the rate of decomposition of hydrazine in a solution of the composition

0.1 mole/liter hydrazine  
0.3 mole/liter disodium hydrogen phosphate  
pH 12.1; adjusted with sodium hydroxide  
at 70°C. The decomposition rate was found to be 300  $\mu\text{mole hydrazine}/\text{cm}^2\text{hr}$ .

By way of comparison, the decomposition rate of the hydrazine under identical experimental conditions on

a sheet of pure nickel (rolled) which was etched at 70°C in 2 N hydrochloric acid was less than 3  $\mu\text{mole hydrazine}/\text{cm}^2\text{hr}$ .

## EXAMPLE 9

5 From an electrolyte of the composition  
0.05 mole/liter nickel (II) sulfate  
10<sup>-3</sup> mole/liter thallium sulfate  
0.6 mole/liter hydrazine  
10 0.4 mole/liter dipotassium hydrogen phosphate  
0.2 mole/liter sodium diphosphate ( $\text{Na}_4\text{P}_2\text{O}_7$ )  
a catalytically active coating was deposited at pH 12.0 (adjusted with sodium hydroxide) and at 70°C as described in Example 8.  
15 The catalytic activity or the alloy coating was 310  $\mu\text{mole hydrazine}/\text{cm}^2\text{hr}$ .

## EXAMPLE 10

20 From an electrolyte of the composition  
0.05 mole/liter nickel (II) sulfate  
10<sup>-3</sup> mole/liter tin (II) chloride  
0.4 mole/liter hydrazine  
0.2 mole/liter sodium diphosphate ( $\text{Na}_4\text{P}_2\text{O}_7$ )  
0.4 mole/liter dipotassium hydrogen phosphate  
25 a catalytically active coating was deposited at pH 11.4 (adjusted with sodium hydroxide) and at 70°C as described in Example 8.

The catalytic activity of the alloy coating was as follows:

30 390  $\mu\text{mole hydrazine}/\text{cm}^2\text{hr}$ .

What is claimed is:

1. In an alkaline chemical nickel plating bath having a surface layer of di-n-butyl ether and a pH above 11 comprising an aqueous solution of a nickel salt, a reducing agent selected from the group consisting of hydrazine and hydrazine salts, a complexing agent and a buffering agent, the improvement of which comprised from 0.05 to 1 mole per liter of at least one water soluble salt of an acid selected from the group consisting of ammonium, sodium, potassium and hydrazonium salts of carbonic acid and phosphoric acid, said bath comprising about 10<sup>-4</sup> to 10<sup>-2</sup> moles per liter of at least one water soluble salt of a metal selected from the group consisting of cobalt, germanium, tin and thallium.

\* \* \* \* \*